

# United States Patent

[11] 3,620,717

[72] Inventors Shozo Sekino;  
Toshiyuki Fujishima; Hiroshi Yada, all of  
Kitakyushu, Japan

[21] Appl. No. 761,474

[22] Filed Sept. 23, 1968

[45] Patented Nov. 16, 1971

[73] Assignee Yawata Iron & Steel Co., Ltd.  
Tokyo, Japan

[32] Priority Sept. 27, 1967

[33] Japan

[31] 42/62125

[56] References Cited

UNITED STATES PATENTS

|           |         |               |          |
|-----------|---------|---------------|----------|
| 3,097,294 | 7/1963  | Kubli.....    | 75/123 R |
| 3,115,406 | 12/1963 | Ballass.....  | 75/124   |
| 3,162,751 | 12/1964 | Robbins ..... | 75/125 X |
| 2,140,237 | 12/1938 | Leitner.....  | 75/128 X |
| 2,289,081 | 7/1942  | Shortell..... | 75/123 X |
| 2,992,148 | 7/1961  | Yeo.....      | 75/123 X |

Primary Examiner—L. Dewayne Rutledge  
Assistant Examiner—Joseph E. Legru  
Attorney—Wenderoth, Lind & Ponack

[54] WELDABLE, ULTRAHIGH TENSILE STEEL  
HAVING AN EXCELLENT TOUGHNESS  
10 Claims, 1 Drawing Fig.

[52] U.S. Cl..... 75/125,  
75/123 J, 75/123 K, 75/128 V, 75/128 W, 75/128  
G, 75/124, 148/31, 148/36

[51] Int. Cl..... C22c 39/50,  
C22c 39/54

[50] Field of Search..... 75/123,  
129, 124, 125, 123 R, 123 K

**ABSTRACT:** A weldable, ultrahigh tensile steel prepared by adding V and Cu to a low-carbon steel containing Ni and Mo, to which there may be further added W, Nb and Ta, characterized by being able to stand a low temperature and possessing a good weldability and an excellent toughness at a very high level of the strength, particularly the toughness in the welding heat-affected zone, said properties being particularly imparted by the addition of V and Cu.





INVENTORS  
Shozo Sekino  
Tohiyuki Fujishima  
Hiroshi Yada

BY,  
Wendell, Lind & Ponack,  
Attn:

## WELDABLE, ULTRAHIGH TENSILE STEEL HAVING AN EXCELLENT TOUGHNESS

### BACKGROUND OF THE INVENTION

#### 1. Field of the Invention

The present invention relates to a high-toughness, ultrahigh tensile steel having an excellent weldability.

#### 2. Description of the Prior Art

Heretofore, it was known that a steel having a yield strength of above 90 kg./mm.<sup>2</sup> and at the same time a relatively good toughness could be obtained, when adding a carbide-forming element to steel containing 4 to 8.5 percent Ni and then subjecting the resultant steel to heat treatments such as quenching and tempering, but it was difficult to obtain a steel which could fulfill the conditions as mentioned in the following, because of the toughness of the welding heat-affected zone being lowered with an increase in the yield strength, that is, for steels to be placed at the service as materials for use in deep sea constructions, particularly such as an outer hull plate of submarine, the following conditions are to be regarded as indispensable:

i. The toughness should be so high as it may stop a further enlargement of cracks of any length occurred at the minimum temperature practically applied and

ii. a welding should be easily feasible and the toughness as above mentioned should be imparted also to the weld.

### SUMMARY OF THE INVENTION

The main object of the present invention is to provide a steel which sufficiently fulfills the conditions as above mentioned, that is, a structural steel material which can well stand a low temperature and has an excellent toughness at a very high level of strength.

Another object of the present invention is to provide a structural steel material which has an excellent weldability and also an excellent toughness particularly of the weld.

And still another object of the present invention will become clear from the following disclosure, making reference to the accompanying drawing, which shows the relations between the Cu content of the steel of the present invention and the yield strength (A), the 2 mm. V-notch Charpy impact value (B) at -80° C. and the 2 mm. V-notch Charpy impact value (C) of a welding thermal cycle reproducing test piece.

The composition ranges of the steel of the present invention, by which the above-mentioned objects can be obtained, are as follows:

|    |                                                  |
|----|--------------------------------------------------|
| C  | 0.04 to 0.15%                                    |
| Si | 0.05 to 0.5%                                     |
| Mn | 0.05 to 1.5%                                     |
| Ni | 4 to 8.5%                                        |
| Mo | 0.25 to 1.5%                                     |
| Cu | 0.4 to 3%, preferably 0.5                        |
|    | to 1.5%                                          |
| V  | 0.04 to 0.15%                                    |
| Al | an amount usually contained in a killed steel    |
|    | the balance being Fe and unavoidable impurities. |

Among the above-mentioned components Mo may be replaced by a double amount of W. Further, to the steel having the composition ranges as above-mentioned there may be added at least an element selected from the group consisting of less than 2 percent Cr, less than 0.10 percent Nb and less than 0.10 percent Ta.

As a rule, the steel of the present invention having the composition as above mentioned is placed at practical services after it has been subjected to the following heat treatments: Immediately after a hot-working or after the hot-working followed by a normalizing at a temperature of 800° to 1,100° C. the steel is quenched from a temperature ranging from 750 to 950° C. and then tempered at a temperature of 500° to 650° C. for 0.5 to 3 hours. Depending upon the composition series it is also possible to omit the quenching.

As above mentioned, in a steel containing 4.0 to 8.5 percent Ni, there occurs a deterioration of the toughness, particularly in the welding heat-affected zone in proportion to an increase in the yield strength. But, with the composition ranges of the present invention, which include especially 0.4 to 3 percent (preferably 0.5 to 1.5 percent) Cu and further 0.04 to 0.15 percent V added together with Cu, the inventors of the present invention succeeded in elevating the strength of the material tempered after quenching and at the same time in remarkably improving the toughness of the welding heat-affected zone thereof. The relations between the Cu content and mechanical properties of the steel will be clearly understood from the attached drawing and the following disclosure.

### BRIEF DESCRIPTION OF THE DRAWING

The drawing involves changes in mechanical properties made in proportion to varying amounts of Cu added to the steel consisting of 0.1 percent C, 0.25 percent Si, 0.2 percent Mn, 6 percent Ni, 0.35 percent Mo, 0.1 percent V, 0.03 percent Al and the balance being Fe and unavoidable impurities, wherein the yield strength indicated by a solid line (A) shows a sudden elevation in the value from about 0.4 percent on and begins to show a lowering tendency after 3 percent, and the 2 mm. V-notch impact value at -80° C. indicated by a dotted line (B) shows a very high value within the range of Cu, covering 0.5 to 1.5 percent and particularly so high as above 18 kg.-mo./cm.<sup>2</sup> at 1 percent of Cu, or even within the ranges of 0.4 to 3.0 percent, the value above 10 kg.-m./cm.<sup>2</sup>, as usually required, which designates an excellent toughness of the steel of the present invention. Further, also the 2 mm. V-notch Charpy impact value at -80° C. indicated by a chain line (C) for test pieces subjected to a welding thermal cycle (with a heat input of 18,000 Jule/cm.) reproducing test shows an increasing value in proportion to an increasing addition of Cu. It is, however, to note that in the case of adding no V neither such high strength nor high toughness of the weld as above mentioned can be obtained, which is clearly seen from a reference steel No. E in the tables 3 and 4 to be shown later indicating the strength and toughness of a steel of the same composition series as that of the steel shown in the drawing, but without the addition of V.

Thus, in the present invention to a steel 4.0 to 8.5 percent Ni steel there are added Cu and V and further Mo or W which may be added to replace a part or a whole of Mo. The steel of the present invention thus obtained by adding the elements as above mentioned is characterized by displaying an excellent toughness at a yield stress of more than 90 kg./mm.<sup>2</sup> due to a secondary hardening by means of the addition of V and Mo or W in a material a welding heat-affected zone by a mutual function of Cu and V.

In the steel of the present invention C is necessary for a strengthening of the steel due to the formation of carbide and for maintaining the proper hardenability. In an amount of less than 0.04 percent the effect of C cannot be displayed, but in an amount of more than 0.15 percent a reduction in the toughness in a welding heat-affected zone is unavoidable. Therefore, the C content is specified to be within the range of 0.04 to 0.15 percent.

Si and Mn are necessary as a deoxidizing agent in making the steel of the present invention. However, Si and Mn an amount of less than 0.05 percent respectively are insufficient to perform the deoxidizing. However, with an amount of more than 0.5 percent Si the toughness is lowered. With an increasing amount of Mn the strength is elevated to some degree and the toughness in a welding heat-affected zone is a little improved, but if above 1.5 percent, there appears remarkably a tendency of deteriorating the toughness of the material tempered after quenching. On the basis of the facts above-mentioned Si is specified to 0.05 to 0.5 percent and Mn 0.05 to 1.5 percent.

Ni is an element necessary to impart a good toughness to a steel material at the high level of strength. In the steel of the

present invention an addition of more than 4 percent Ni is necessary in order to keep the toughness which is more than 90 kg./mm.<sup>2</sup> and is to fulfill the conditions as above mentioned. But, with an addition of more than 8.5 percent a specially remarkable improvement in the toughness can not be expected. Therefore, the addition of Ni is limited to 4 to 8.5 percent.

Mo and V are a carbide-forming element respectively which has a function of effecting a remarkable secondary hardening by a tempering treatment within a temperature range of 500° to 650° C. and further V has the function of improving the toughness in the welding heat-affected zone under the coexistence with Cu. In the steel of the present invention a sufficient strength can not be obtained by the addition of Mo in an amount of less than 0.25 percent and V in an amount of less than 0.04 percent. On the other hand, if the addition of Mo and V exceeds 1.5 percent and 0.15 percent respectively, the effects thereof reach the saturation and there appear rather tendencies of the steel being softened and the weldability being deteriorated. Therefore, Mo is defined to be in the range of 0.25 to 1.5 percent and V in the range of 0.04 to 0.15 percent. Further, a part or whole of Mo may be replaced by W.

Cu shows a remarkable effect of preventing the embrittlement of the welding heat-affected zone, particularly by the mutual function with V in the Ni-steel, the strength of which has been increased by carbides of Mo and V as above mentioned. In the steel of the present invention an addition of at least 0.4 percent Cu is absolutely necessary. That is, with an increasing amount of Cu above 0.4 percent its effect of preventing the embrittlement of the welding heat-affected zone becomes remarkable, simultaneously accompanied with the effect of increasing the strength of the steel to some degree. However, if the amount of Cu exceeds 1.0 percent, there appears a tendency of lowering the toughness of the material tempered after quenching, and particularly, above 3 percent, the said tendency becomes notable. Therefore, the amount of Cu is specified to the range of 0.4 to 3.0 percent, preferably 0.5 to 1.5 percent.

Cr has an effect as carbide-forming element of elevating the

steel by causing fine carbonitride to precipitate mainly during a hot-working and of refining austenitic crystal grains thereby. However, if the addition of Nb+Ta exceeds 0.10 percent, the toughness is rather deteriorated because of large precipitates of carbonitride being formed in grain boundaries. Thus, the addition of Nb+Ta is limited to less than 0.10 percent.

W has substantially the same effect as Mo in forming carbide. In the steel of the present invention a part or whole of Mo may be replaced by a double amount of W without producing any difference in characteristics of the steel.

Al has an effect of refining crystal grains even with an addition of such a small amount, as is to be added to the steel as a deoxidizer. However, in the steel of the present invention the addition of Al may be dispensed with. However, if it is to be added, it may be added in an amount of less than 0.07 percent, that is, an amount usually contained in a killed steel.

The steel of the present invention shall be explained more in detail on the basis of examples.

Alloy steel samples Nos. 1 to 15 having the chemical compositions as shown in table 1 within the ranges specified by the present invention were prepared by melting and then subjected to a slabbing and a hot-rolling to make steel plates having a thickness of 13 mm. respectively therefrom. Each steel plate was then normalized at a temperature of 850° C. and thereupon was quenched in water after heated to a temperature of 800° to 900° C. The quenching was followed by a tempering at a temperature of 600° C. or 625° C. The mechanical properties of each steel plate thus quenched and tempered were shown in table 2. As the results of various investigations on said samples to measure small-sized 2 mm. V-notch impact values on conditions as shown in table 2, (1) and (2) it has been confirmed that in the case of (1) the impact value is satisfactory, if it exceeds 8.0 kg.-m./cm.<sup>2</sup> at a temperature lower by more than 20° C. than the minimum temperature practically applied, and in the case of (2) the impact value is satisfactory if it exceeds 4.0 kg.-m./cm.<sup>2</sup> at a temperature lower by 20° C. than the minimum temperature practically applied to test pieces subjected to a welding thermal cycle

reproduction test.

TABLE 1

| Sample No. of the steel of the present invention | Composition (percent) |      |      |      |       |      |      |         |               |
|--------------------------------------------------|-----------------------|------|------|------|-------|------|------|---------|---------------|
|                                                  | C                     | Si   | Mn   | Ni   | Mo    | V    | Cu   | Sol. Al | Others        |
| 1.                                               | 0.048                 | 0.27 | 0.22 | 5.94 | 0.81  | 0.11 | 0.42 | 0.041   |               |
| 2.                                               | 0.14                  | 0.11 | 0.18 | 6.02 | 0.31  | 0.15 | 0.48 | 0.051   |               |
| 3.                                               | 0.09                  | 0.17 | 0.05 | 6.03 | 0.35  | 0.09 | 0.48 | 0.029   | Cr, 1.01      |
| 4.                                               | 0.041                 | 0.22 | 1.36 | 5.41 | 0.59  | 0.10 | 1.44 | 0.034   | Cr, 1.04      |
| 5.                                               | 0.095                 | 0.24 | 0.47 | 4.29 | 0.54  | 0.10 | 0.97 | 0.012   |               |
| 6.                                               | 0.065                 | 0.25 | 0.22 | 8.13 | 0.28  | 0.11 | 0.43 | 0.048   |               |
| 7.                                               | 0.072                 | 0.27 | 0.22 | 6.11 | 0.40  | 0.11 | 0.42 | 0.042   |               |
| 8.                                               | 0.10                  | 0.28 | 0.24 | 4.88 | 0.33  | 0.05 | 1.54 | 0.013   |               |
| 9.                                               | 0.093                 | 0.28 | 0.19 | 5.95 | 0.35  | 0.10 | 2.86 | 0.002   |               |
| 10.                                              | 0.12                  | 0.42 | 0.18 | 6.02 | 0.36  | 0.15 | 0.48 | 0.057   | Cr, 1.08      |
| 11.                                              | 0.09                  | 0.29 | 0.25 | 4.80 | 0.35  | 0.10 | 0.51 | 0.036   | Cr, 1.45      |
| 12.                                              | 0.13                  | 0.15 | 1.30 | 4.88 | 0.51  | 0.05 | 0.51 | 0.044   | Cr, 1.45      |
| 13.                                              | 0.084                 | 0.27 | 0.22 | 6.17 | 0.30  | 0.11 | 0.42 | 0.042   | {Nb+Ta, 0.036 |
| 14.                                              | 0.088                 | 0.29 | 0.22 | 6.05 | ----- | 0.11 | 0.42 | 0.046   | W, 0.48       |
| 15.                                              | 0.080                 | 0.28 | 0.32 | 6.05 | ----- | 0.10 | 0.47 | 0.037   | W, 2.05       |

strength of the steel of the present invention. However, as stronger carbide-forming elements such as Mo and V are used in the steel of the present invention, the effect of Cr as the carbide-forming element is not so much expected. Moreover, as Cr has a tendency of deteriorating the weldability, the addition of Cr may be dispensed with. But, also the addition of Cr is effective in such a case, where a high hardenability is required when the contents of such elements as C, Mn and Mo, which elevate the hardenability of steel, are those near the lower limits of the respective ranges within the composition of the steel of the present invention. However, even in this case, the addition of Cr is to be limited to less than 2.0 percent, as it has a tendency of lowering the toughness of the material tempered after quenching, because of a huge carbide being formed thereby, if it is added in an amount more than required.

Nb and Ta are a strong carbonitride-forming element respectively, which has an effect of elevating the toughness of

TABLE 2

| Sample No. of the steel of the present invention | Yield strength, kg./mm. <sup>2</sup> | V-notch Charpy impact value at -80° C., kg.-m./cm. <sup>2</sup> | V-notch Charpy impact value at -80° C., kg.-m./cm. <sup>2</sup> | thermal cycle test (with heat input of 18,000 Jule/cm. <sup>2</sup> ) kg.-m./cm. <sup>2</sup> |
|--------------------------------------------------|--------------------------------------|-----------------------------------------------------------------|-----------------------------------------------------------------|-----------------------------------------------------------------------------------------------|
|                                                  |                                      |                                                                 |                                                                 |                                                                                               |
| 1.                                               | 110                                  | 11.0                                                            | 11.0                                                            | 7.8                                                                                           |
| 2.                                               | 103                                  | 19.8                                                            | 19.8                                                            | 6.2                                                                                           |
| 3.                                               | 101                                  | 21.2                                                            | 21.2                                                            | 4.5                                                                                           |
| 4.                                               | 98                                   | 17.7                                                            | 17.7                                                            | 9.5                                                                                           |
| 5.                                               | 108                                  | 9.8                                                             | 9.8                                                             | 8.1                                                                                           |
| 6.                                               | 107                                  | 16.0                                                            | 16.0                                                            | 9.4                                                                                           |
| 7.                                               | 115                                  | 9.5                                                             | 9.5                                                             | 8.2                                                                                           |
| 8.                                               | 96                                   | 21.8                                                            | 21.8                                                            | 6.0                                                                                           |
| 9.                                               | 106                                  | 11.8                                                            | 11.8                                                            | 9.6                                                                                           |
| 10.                                              | 104                                  | 18.0                                                            | 18.0                                                            | 6.0                                                                                           |
| 11.                                              | 94                                   | 21.2                                                            | 21.2                                                            | 4.3                                                                                           |
| 12.                                              | 98                                   | 23.4                                                            | 23.4                                                            | 4.2                                                                                           |
| 13.                                              | 117                                  | 10.3                                                            | 10.3                                                            | 6.5                                                                                           |
| 14.                                              | 122                                  | 9.1                                                             | 9.1                                                             | 7.2                                                                                           |
| 15.                                              | 112                                  | 10.1                                                            | 10.1                                                            | 7.3                                                                                           |

As is shown in table 2, all of the samples show the yield strength of more than 90 kg./mm.<sup>2</sup> and fulfill the conditions as above mentioned. Among these samples Nos. 1 and 4, which contain a smaller amount of C respectively and Nos. 1, 4, 5, 7, 14 and 15 which contain a larger amount of Mo (or W) respectively show such very high impact values at -80° C. for the test pieces subjected to a thermal cycle reproduction test as of more than 7 kg.-m./cm.<sup>2</sup>, implying an excellent toughness of these samples. This is one of the most characteristic features of the present invention.

At last, in order to evidence that the composition ranges of the steel of the present invention should absolutely be kept as specified by the present invention, there are shown in table 3 some examples of steels having composition ranges different from those of the steel of the present invention in that in one of these examples there is lacking in one of elements essential for the steel of the present invention and in another of them there is added another of these elements too much or too little, and the results of the same tests as made in table 1 are shown in table 4.

TABLE 3

| Reference steel No. | Composition (percent) |      |      |      |      |      |      |        |          |
|---------------------|-----------------------|------|------|------|------|------|------|--------|----------|
|                     | C                     | Si   | Mn   | Ni   | Mo   | V    | Cu   | Si. Al | Others   |
| A                   | 0.101                 | 0.24 | 0.06 | 3.75 | 0.57 | 0.05 | 0.48 | 0.022  |          |
| B                   | 0.095                 | 0.24 | 2.48 | 4.65 | 0.30 | 0.14 | 0.5  | 0.05   |          |
| C                   | 0.10                  | 0.25 | 0.23 | 4.80 | 0.33 | 0.14 | —    | 0.014  | Cr, 1.05 |
| D                   | 0.10                  | 0.28 | 0.23 | 5.22 | 0.16 | 0.13 | 0.51 | 0.038  | Cr, 1.04 |
| E                   | 0.10                  | 0.29 | 0.25 | 4.88 | 0.34 | —    | 0.47 | 0.036  | Cr, 0.22 |

TABLE 4

| Reference steel No. | Yield strength, kg./mm. <sup>2</sup> | V-notch Charpy impact value at -80° C., kg.-m./cm. <sup>2</sup> |                                     | heat input of 18,000 Jule/cm. <sup>2</sup> | kg.-m./cm. <sup>2</sup> |
|---------------------|--------------------------------------|-----------------------------------------------------------------|-------------------------------------|--------------------------------------------|-------------------------|
|                     |                                      | at -80° C., kg.-m./cm. <sup>2</sup>                             | at -80° C., kg.-m./cm. <sup>2</sup> |                                            |                         |
| A                   | 99                                   | 12.8                                                            | —                                   | 1.0                                        |                         |
| B                   | 103                                  | 5.8                                                             | —                                   | 2.6                                        |                         |
| C                   | 102                                  | 11.7                                                            | —                                   | 2.8                                        |                         |
| D                   | 84                                   | 23.6                                                            | —                                   | 2.4                                        |                         |
| E                   | 88                                   | 26.0                                                            | —                                   | 3.0                                        |                         |

No. A contains a smaller amount of Ni, No. B a larger amount of Mn and No. C contains no Cu. All of these three samples show insufficient impact values of test pieces subjected to a welding thermal cycle reproduction test. No. D has a smaller amount of Mo and No. E contains no V, and both samples are not only low in the strength, as either shows the yield strength of less than 90 kg./mm.<sup>2</sup>, but also low in the toughness, as are shown with the impact values of test pieces subjected to a welding thermal cycle reproduction test of below 4 kg.-m./cm.<sup>2</sup>, which means that the coexistence of Cu with V is indispensable. It is evident from the foregoing that the composition ranges as above mentioned can produce a steel as that of the present invention which is distinguished at the same time by an excellent toughness and weldability and particularly is fit for the uses which the present invention has for its object.

The examples above mentioned do not designate those which limit the scope of the present invention. Obviously

many modifications and variations of the present invention are possible within the composition ranges above mentioned. It is therefore, to be understood that within the scope of the composition ranges as above mentioned the invention may widely be practiced otherwise than as specially described

5 What is claimed is:

1. A weldable ultrahigh tensile steel having a yield strength of above 90 kg./mm.<sup>2</sup> and at the same time an excellent toughness at a low temperature and good weldability comprising

10 0.04 to 0.15 percent by weight C  
0.05 to 0.5 percent by weight Si  
0.05 to 1.5 percent by weight Mn  
4.0 to 8.5 percent by weight Ni  
15 0.25 to 3.0 percent by weight Mo  
0.04 to 0.15 percent by weight V  
0.4 to 3.0 percent by weight Cu  
the balance being Fe and unavoidable impurities.

2. The steel claimed in claim 1, wherein Al is added in an 20 amount of less than 0.07 percent by weight.

3. The steel claimed in claim 1, wherein a part of Mo is replaced by a double amount of W.

4. The steel claimed in claim 1, wherein a whole of Mo is replaced by a double amount of W.

5. The steel claimed in claim 1, wherein the steel is quenched from a temperature ranging from 750° C. to 950° C. and then tempered at a temperature of 500° to 650° C.

6. A weldable steel ultrahigh tensile strength having a yield strength of above 90 kg./mm.<sup>2</sup> and at the same time an excellent toughness at a low temperature and good weldability, comprising

40 0.04 to 0.15 percent by weight C  
0.05 to 0.5 percent by weight Si  
0.05 to 1.5 percent by weight Mn  
4.0 to 8.5 percent by weight Ni  
0.25 to 3.0 percent by weight Mo  
0.4 to 3.0 percent by weight Cu  
0.04 to 0.15 percent by weight V  
less than 2.0 percent by weight Cr,  
50 the balance being Fe and unavoidable impurities.

7. The steel claimed in claim 6, wherein Al is added in an amount of less than 0.07 percent by weight.

8. The steel claimed in claim 6, wherein a part of Mo is replaced by a double amount of W.

9. The steel claimed in claim 6, wherein a whole of Mo is replaced by a double amount of W.

10. The steel claimed in claim 6, wherein the steel is quenched from a temperature ranging from 750° to 950° C. and then tempered at a temperature of 500° to 650° C.

\* \* \* \* \*